

# UNITED STATES PATENT OFFICE.

EDWARD A. COOK, OF GIATTO, WEST VIRGINIA, ASSIGNOR OF ONE-THIRD  
TO TIMOTHY W. PATTON, OF BLUEFIELD, WEST VIRGINIA.

## SHOE-POLISHING COMPOUND.

No. 820,392.

Specification of Letters Patent.

Patented May 15, 1906.

Application filed October 14, 1905. Serial No. 282,848.

*To all whom it may concern:*

Be it known that I, EDWARD A. COOK, a citizen of the United States, residing at Giatto, in the county of Mercer and State of West Virginia, have invented a new and useful Shoe-Polishing Compound, of which the following is a specification.

This invention relates to a compound for polishing boots, shoes, harness, and leather of all kinds, and has for its object to provide a compound of this character particularly adapted as a dressing and preservative for patent and enamel shoes and which when applied to the shoes will render the leather soft, pliable, and impervious to moisture and give the same a brilliant and lasting polish.

With these and other objects in view the invention consists in a compound or dressing formed of the following ingredients in the proportions stated: castor-oil, seven pints; sperm-oil, one pint; lemon-extract, two ounces, and powdered charcoal, six ounces.

In preparing the compound the castor-oil and sperm-oil are poured into a suitable receptacle, together with the extract of lemon, after which the finely-powdered charcoal is added and the several ingredients thoroughly mixed or stirred until the parts are well blended. The compound thus formed may be put up in bottles of convenient sizes for future use and may be applied to the shoes with a brush, sponge, or in any other suitable manner. The sperm-oil fills the pores of the

leather and renders the same soft and pliable, while the castor-oil preserves the surface of the leather and holds the oil in the pores of the same. The lemon extract gives the shoe the desired shine or polish, and the charcoal colors the liquid and assists in keeping the surface of the leather glossy.

The above compound or dressing applied in the manner stated will preserve the leather and effectually prevent the enamel from cracking or peeling and at the same time render the leather moisture-proof and give the same a smooth glossy appearance.

Having thus described the invention, what is claimed is—

1. The herein-described compound for polishing and preserving boots and shoes the same consisting of castor-oil, sperm-oil, extract of lemon and powdered charcoal, combined in the manner specified.

2. The herein-described compound for polishing and preserving boots and shoes, the same consisting of castor-oil seven pints, sperm-oil one pint, extract of lemon two ounces, and powdered charcoal six ounces.

In testimony that I claim the foregoing as my own I have hereto affixed my signature in the presence of two witnesses.

EDWARD A. COOK.

Witnesses:

R. N. VERMILLION,  
ELMER BAILEY.